

# UNITED STATES PATENT OFFICE.

FRANK C. AXTELL, OF NEW YORK, N. Y.

## LIQUID FUEL.

1,204,638.

Specification of Letters Patent. Patented Nov. 14, 1916.

No Drawing.

Application filed September 5, 1916. Serial No. 118,384.

To all whom it may concern:

Be it known that I, FRANK C. AXTELL, a citizen of the United States, and resident of New York city, borough of Manhattan, in the county of New York and State of New York, have invented certain new and useful improvements in Liquid Fuel, of which the following is a specification.

The object of my invention is to provide a liquid fuel particularly adapted for use in the production of a combustible mixture for the operation of internal combustion engines, which fuel may be used as a substitute for gasoline in such engines, a further object being to enable the utilization in the fuel of a cheap base, whereby fuel may be produced at a relatively low cost.

In carrying out my invention I make a mixture comprising a light hydrocarbon oil, (such as kerosene), a light hydrocarbon distillate, and alcohol, with which is combined what I term a "mixing" or "combining" agent comprising a liquid, or mixture of liquids, which is soluble or miscible with each of the constituent liquids above named in all proportions.

My improved liquid fuel may be produced as follows: To two volumes of hydrocarbon oil, such as kerosene, preferably that which is known in commerce as "export oil," (commercial kerosene having a flash-point of 100° to 110° F.) I add one volume of a light paraffin distillate boiling at about 60° to 80° C., or the same volume of a light distillate, such as is obtained by "cracking" or decomposing paraffin oils in heated retorts, and to such mixture of hydrocarbon oil, (export oil), and light distillate, I add one volume of alcohol of about 95 volume per cent. Under such conditions the alcohol does not mix with the aforesaid mixture of oil and light distillate, and the whole mixture would separate into two strata, one of which consists almost entirely of the hydrocarbons and the other of alcohol and water, and in order to cause them to combine to form a homogeneous mixture I add thereto a certain proportion of the "mixing" or "combining" agent above referred to. Such mixing or combining agent may consist of any suitable liquid or mixture of liquids which is soluble or miscible in all proportions with each of the constituent liquids above named. Thus, a liquid which is soluble or miscible in all proportions in "export oil", in either of the

light distillates described, and in alcohol of 95 volume per cent., would constitute a "mixing" or "combining" agent, within the scope of the appended claims. It will be evident to those skilled in this art that there are various liquids which will fulfil the requirements and which possess the properties I have described regarding the said "mixing" or "combining" agent, and as specific illustrations I may mention commercial anhydrous fusel oil and commercial anhydrous amyl alcohol, either of which, when added in certain proportion to the aforesaid mixture of hydrocarbons, (such as export oil and light distillate, and alcohol of 95 volume per cent.), causes such liquids to mix perfectly, the resulting mixture being a homogeneous liquid fuel, which will remain mixed and not separate. As an example of the proportion of the aforesaid "mixing" or "combining" agent which may be mixed with the aforesaid hydrocarbons and alcohol, it will be found that four-tenths (0.4) volume of anhydrous fusel oil or anhydrous amyl alcohol mixed with the above described mixture of two volumes of export oil, one volume of light paraffin distillate or of cracked distillate, and one volume of alcohol at 95 volume per cent., will produce the homogeneous mixture described.

While I have mentioned examples of proportions of the various ingredients utilized in the production of my improved liquid fuel, it will be understood that the proportions mentioned may be varied in order to meet the desired requirements, or for the production of my improved liquid fuel of varying grades or volatility, or having the most desirable properties for the use to which it is to be applied.

Some of the advantages of my new liquid fuel, when compared with ordinary commercial gasoline of to-day, are that my fuel produces a more perfect combustion in the engine cylinders, yields considerably more power, is capable of taking up or dissolving small quantities of water (up to about three-fourths of one per cent.), without separating, thus eliminating one of the inherent troubles in such use of the aforesaid gasoline, and further, that my improved fuel may be produced at a relatively low cost. When my improved liquid fuel is used for the production of a combustible mixture for internal combustion engines, it may be sup-

plied to the engine through a carburetor in the ordinary manner of using gasoline for such purpose.

While I have referred to my improved liquid composition as adapted as a liquid fuel, which, when mixed with air in proper proportions, would serve as a mixture for use in internal combustion engines, it will be understood that such a composition may 10 be utilized for any other desired purpose to which it may be found applicable.

While I refer herein to anhydrous fusel oil, it will be understood that I intend by such term to include anhydrous amyl alcohol, and where I have referred to a "light distillate" I intend the term to include a hydrocarbon distillate, whether of the light paraffin series or such as is obtained by cracking or decomposing paraffin oils in 15 heated retorts, the term being intended by me to include hydrocarbons having a gravity lighter than kerosene oil.

Having now described my invention what I claim is:

1. A liquid fuel comprising hydrocarbon oil, a light hydrocarbon distillate, an alcohol normally insoluble in the aforesaid ingredients, and a mixing or combining agent for causing the intimate mixture of said ingredients, the several components of the mixture being in such proportions as to flash 20 in the cylinder of an internal combustion engine at normal temperatures.

2. A liquid fuel comprising about two volumes of kerosene, about one volume of a light hydrocarbon distillate, about one volume of alcohol (about 95 volume per cent.), and about four-tenths (0.4) volume of anhydrous fusel oil.

Signed at New York city, in the county of New York and State of New York this 25 second day of September, A. D. 1916.

FRANK C. AXTELL.